

Aug. 9, 1932.

W. C. SMITH

1,870,470

CONCENTRATION OF BISMUTH ALLOY

Filed June 4, 1930



Fig:1.



Fig:2.

INVENTOR

Walter C. Smith

BY

Paul R. Ames  
ATTORNEY

## UNITED STATES PATENT OFFICE

WALTER C. SMITH, OF MAPLEWOOD, NEW JERSEY, ASSIGNOR TO CERRO DE PASCO COPPER CORPORATION, OF NEW YORK, N. Y., A CORPORATION OF NEW YORK

## CONCENTRATION OF BISMUTH ALLOY

Application filed June 4, 1930. Serial No. 459,180.

This invention relates to the recovery or treatment of bismuth and more particularly to the concentration by selective oxidation of alloys or metal mixtures containing bismuth.

In the concentration by selective oxidation of bismuth alloys, or metal mixtures containing bismuth, it has been the practice to submit the alloy or mixture to cupellation by subjecting the surface of the molten metal to the action of a stream of air directed across the surface of such metal. Selective oxidation of bismuth alloys has also been conducted by introducing air into the molten alloy through pipes having their ends submerged in the molten metal.

By following either of the above methods, the oxidation is relatively slow and it is necessary to supply heat to the furnace by burning fuel, in order to maintain the temperature of the metal and slag sufficiently high to allow the reactions to proceed. When the air is passed into the molten mass through pipes projecting into the metal, the deterioration of the pipes is very rapid, with a resultant excessive cost and a very rapid addition of impurities to the molten slag. Iron pipes are generally used and the iron acts as a reducing agent on the oxides in the molten slag, thereby retarding the speed of the concentration of bismuth. Furthermore, in following this procedure it is impracticable to use a sufficient number of pipes to supply an adequate amount of oxygen to the molten mass.

It is an object of this invention to avoid the above difficulties and to provide an improved method and means for concentrating the bismuth in metal mixtures containing it. A further object of this invention is to provide a means and method whereby such concentration may be conducted without the use of fuel in the furnace. Other objects will become apparent.

My improved process is carried out by oxidizing the molten mixture of metals in a basic lined furnace of the tilting or rotating type. The furnace may be of any suitable construction but for the purpose of illustration the invention will be described in

connection with a horizontal rotatable furnace.

In the drawing, Figure 1 is a vertical section through the axis of the furnace and Figure 2 is a section taken on the line 2—2 of Figure 1. The furnace 1, having a basic lining 2, is rotated upon the rollers 3, 3 in a clockwise direction, as viewed in Figure 2, to a position in which the tuyères 4 terminate above the level to be occupied by the molten metal. The metal is then placed in the furnace and the latter is fired by the burners 5, 5 until the metal is reduced to a molten state. Air is then admitted to the tuyères under pressure through the supply pipe 6 which is pivoted at 7, and the furnace is then rotated in a counter-clockwise direction to the position shown in the drawing. The air is forced through the molten metal until the concentration by selective oxidation is completed, the gaseous products of combustion being led to the stack through the outlet 8. The ends of the tuyères 4 should be protected from the molten metal and slag by a suitable lining material.

By following this procedure, the lead, tin, arsenic, sulphur and antimony present in the molten mass will be oxidized and may be separated as fused slag or as fumes. The oxidation of these impurities may be conducted so rapidly by this method that the resultant heat will maintain the molten mass at the required temperature. A layer of slag accumulates on the surface of the molten metal and may be removed from time to time by rotating the furnace and pouring it off through the opening 8. Additional metal may be added to the furnace during the course of the operation and the heat generated by the oxidation will serve to melt this added metal and to oxidize the impurities in it.

The temperature of the metal in the furnace may be controlled by regulating the air supply and the quantity of metal added to the furnace. For example, if the furnace becomes too hot the air supply may be cut down by a valve (not shown) in the supply pipe 6, and/or additional metal may be added to the furnace.

In using my improved process in a furnace having the dimensions of about 3 by 6 feet, a charge consisting of a bullion containing about 10% bismuth may be concentrated 5 to 65% bismuth in about 24 hours as compared with 60 to 72 hours required to concentrate the same charge by the usual procedure. Furthermore, a saving of about 450 gallons of oil, or the equivalent of other fuel, is ac- 10 complished at the same time.

It is apparent that modifications of my invention may be made to adapt it to different uses and it is not intended to limit it to the particular embodiment described and 15 illustrated.

What I claim is:

1. A process for concentrating bismuth in a bismuth bullion containing as an impurity an element of the group comprising lead, tin, 20 arsenic, sulphur and antimony, comprising passing air through the molten mass at such a rate that the oxidation of impurities in the bullion will generate sufficient heat to maintain the metal in a molten state.
2. In the concentration of bismuth in a bismuth bullion, containing as an impurity an element of the group comprising lead, tin, arsenic, sulphur and antimony, the steps comprising melting the bismuth bullion and 25 passing air through the molten metal to oxidize the impurities and maintain the mass in a molten state, and separating the oxidized impurities with the slag.
3. A process for concentrating bismuth in 30 a bullion containing lead and bismuth, comprising heating the bullion to reduce it to a molten state and thereafter bubbling air through it at such a rate that the selective oxidation of the metals associated with the bismuth will maintain the mass in a molten state.
4. In the concentration of bismuth in a bullion containing lead and about 10% bismuth, the steps comprising heating the mass 45 to reduce it to a molten condition and thereafter cutting off the external heat and passing air through the molten mass at such a rate as to maintain it in a molten condition.
5. A process for concentrating bismuth in 50 a bullion containing lead and bismuth, comprising heating the bullion to reduce it to a molten mass and thereafter bubbling air through it at such a rate that the selective oxidation of metals associated with the bismuth will maintain the mass in a molten condition, removing the slag containing the oxidized metals separated from the bismuth and adding further bullion to the molten mass 55 and melting the added bullion by the heat from the oxidation.

In testimony whereof, I have signed my name to this specification this 26th day of May, 1930.

WALTER C. SMITH.